

1

2,871,197

## RESISTANCE MATERIAL FOR FIRE DETECTOR ELEMENT

Ronald MacIntyre, North Arlington, and Leonard Junior Sheakley, Verona, N. J., assignors to Specialties Development Corporation, Belleville, N. J., a corporation of New Jersey

No Drawing. Application October 26, 1954  
Serial No. 464,907

2 Claims. (Cl. 252—518)

The present invention relates to fire detector elements, and, more particularly, to a core composed of a resistance material adapted to be utilized in connection with such elements.

The invention is concerned with fire detector elements comprising two or more spaced apart conductors of electricity having therebetween a core composition of such a resistance at normal temperatures that, in effect, it insulates the conductors, and of such a resistance at a predetermined higher temperature that it becomes a conductor of electricity between the conductors and enables sufficient current to pass through the conductors to operate a device for controlling a fire alarm and/or fire extinguishing circuit. For example, as shown in United States Letters Patent No. 2,586,252, the elements may be in the form of a cable-like structure adapted to be placed in a space where a fire is to be detected. This structure comprises a metallic tube through which electrically conductive wires extend which are separated from each other and the tube by a suitable resistance material of the foregoing character.

More specifically, the present invention is primarily concerned with improving this resistance material in a manner to more accurately predetermine the temperature at which it is rendered conductive in response to the heat of a fire, whereby current can flow through the conductors to operate an electrical device.

Accordingly, an object of the present invention is to provide an improved resistance material of the character indicated herein.

Another object is to provide such a material which becomes electrically conductive practically instantaneously when heated to a relatively low, predetermined temperature.

A further object is to provide such a material which is economical to prepare, is reliable in operation, and is fully adapted for repeated use without change in its responsive characteristic.

Other and further objects of the invention will be obvious upon an understanding of the illustrative embodiment about to be described, or will be indicated in the appended claims, and various advantages not referred to herein will occur to one skilled in the art upon employment of the invention in practice.

In accordance with the present invention, it has been found that the foregoing objects can be accomplished by utilizing a resistance material, comprising manganese dioxide, zirconium silicate, a frit and an inert ceramic body.

The manganese dioxide and zirconium silicate may be of a chemically pure or technical grade.

The frit may be any of the well known frits described in the literature which are generally utilized in providing the so called enamel base coating on metallic kitchenware and the like. This frit when used in a sufficient amount, serves as a body or carrier for the manganese dioxide to place the composition in glass phase, but its

2

chemical composition does not materially affect the electrical properties of the composition about to be described.

By way of example such a frit may be prepared by melting, solidifying and grinding a mixture comprising

|                | Percent by weight |
|----------------|-------------------|
| Feldspar       | 32.0              |
| Flint          | 11.5              |
| Borax          | 37.5              |
| Soda ash       | 6.0               |
| Sodium nitrate | 4.0               |
| Fluorspar      | 9.0               |

Twenty five parts by weight of this frit are then combined with seventy five parts by weight of a mixture consisting of 90% steatite and 10% flour.

The manganese dioxide, zirconium silicate, frit, steatite and flour are dry blended, and sufficient water is added to make the mixture plastic. The plastic mass is then extruded onto the wires and is baked at about 2,000° F. to fuse the same to the wires as the water is driven off and the flour is burnt out.

It has been discovered that the amount of manganese dioxide in the composition determines the temperature at which the core becomes conductive. For example, a mixture of about 50% manganese dioxide, about 12.5% frit, about 33.75% steatite and about 3.75% flour, to which about 4 parts by weight of zirconium silicate have been added, produces cores which become conductive at a temperature of about 300° F.

It has further been discovered that the zirconium silicate acts as a fluxing agent to provide for good adherence of the core composition to the wires, gives the core composition a high structural strength, particularly high green strength, and gives the core composition a high initial resistance which drops sharply at the predetermined temperature to render the composition conductive.

The following formula illustrates a specific core composition in accordance with the present invention.

|                    | Parts by weight |
|--------------------|-----------------|
| Manganese dioxide  | 50              |
| Frit               | 12.5            |
| Steatite           | 33.75           |
| Flour              | 3.75            |
| Zirconium silicate | 4               |

A composition was produced from these materials and was applied to two-wire temperature sensing elements in the foregoing described manner. The wires were composed of "Inconel," and had a length of ten feet and a diameter of .010 inch. This core had a diameter of .058 inch, and the wires were disposed therein in parallel relation about .010 inch apart throughout their length. These sensing elements had an infinite resistance at 70° F. which dropped sharply to about 5,000 ohms when the composition was heated to 300° F. thereby enabling sufficient direct current or alternating current to flow through the wires to effect operation of an electrical device for giving an indication that the aforementioned temperature condition existed.

From the foregoing description, it will be seen that the present invention provides a composition for temperature sensing elements which has desirable physical and electrical properties, and, in particular, has a sharp resistance drop at a selected temperature to give a rapid and reliable indication that such temperature has been detected.

It will be understood that the details and examples hereinbefore set forth are illustrative only and that the invention as broadly described and claimed is in no way limited thereby.

We claim:

1. A resistance material consisting essentially of about 50 parts by weight of manganese dioxide, about 4 parts by weight of zirconium silicate, about 12.5 parts by weight of a frit, and about 33.75 parts by weight of steatite.

2. A resistance material extrudable as a plastic mass onto electrical conductors and adapted to be fused thereon, said material consisting essentially of about 50 parts by weight of manganese dioxide, about 4 parts by weight of zirconium silicate, about 12.5 parts by weight of a frit, about 33.75 parts by weight of steatite, about 3.75

parts by weight of flour and sufficient water to render the material extrudable.

References Cited in the file of this patent

UNITED STATES PATENTS

2,495,867 Peters ----- Jan. 31, 1950  
2,587,916 Squier ----- Mar. 4, 1952

OTHER REFERENCES

"Ceramic Industry," Jan. 1954, page 133.